

1,297,009.

G. PRIFOLD.  
PROCESS OF MAKING FLOOR COVERINGS.  
APPLICATION FILED DEC. 12, 1917.

Patented Mar. 11, 1919.

*Fig. 1.*



Inventor:  
George Prifold  
by his Attorneys  
Housont Housont

# UNITED STATES PATENT OFFICE.

GEORGE PRIFOLD, OF LINWOOD, PENNSYLVANIA, ASSIGNOR TO THE CONGOLEUM COMPANY, OF PHILADELPHIA, PENNSYLVANIA, A CORPORATION OF PENNSYLVANIA.

## PROCESS OF MAKING FLOOR-COVERINGS.

1,297,009.

Specification of Letters Patent. Patented Mar. 11, 1919.

Application filed December 12, 1917. Serial No. 206,824.

*To all whom it may concern:*

Be it known that I, GEORGE PRIFOLD, a citizen of the United States, and a resident of Linwood, county of Delaware, State of 5 Pennsylvania, have invented certain Improvements in Processes of Making Floor-Coverings, of which the following is a specification.

One object of my invention is to improve 10 the process of making a rug of the type having a felt base and a printed pigment surface.

A further object of the invention is to proportion the base and the printed surface 15 so that they will have the same coefficient of expansion and contraction.

A still further object of the invention is to dispense with sizing in preparing the 20 felt base for the printed surface so as to allow the base to expand and contract with the painted surface.

Figure 1 is a view of a rug made in accordance with my invention, and

Fig. 2 is a perspective view showing the 25 layers cut away and exaggerated to illustrate different steps in the process of manufacturing the rug.

I first make body 1 of dry felt, preferably from cotton rags, although it may be made 30 from other cotton waste, or other suitable material. I saturate the felt with a substance which will thoroughly impregnate it, making it proof against moisture and pliable as at 2, Fig. 2. The substance I prefer to use is a semi-solid bituminous material, which, in the present instance, consists of a petroleum flux-oil and a residual pitch derived from asphaltic or semi-asphaltic base oils, but other hydrocarbons 35 may be used without departing from the spirit of the invention. The material is brought to a temperature of about 500° F. and is then placed in a saturating kettle of such a size and diameter as to allow the 40 felt to be passed through it at a given speed, the material in the kettle having a temperature of about 350° F. during the saturating process, and as the dry felt is 45 passed through the liquor it will be thoroughly impregnated and the surface of the felt will be in such a condition that the 50 paint coatings can be applied thereto when the felt is dry. The material is allowed to cool to a certain degree and while still warm 55 that surface of the felt which is to form

the back of a rug is coated with a suitable paint composition, as at 3. The material is then subjected to heat and also to an air blast to set the coating and to season the felt. After the back coating is dry, then 60 the face of the felt is also treated in the same manner. The back coating is a preparation of linseed oil, naphtha and a pigment, and when the surface is passed over a hot roller the naphtha is evaporated and 65 when the surface is subjected to an air blast the coating is set and dried. The same combination of linseed oil, naphtha and a pigment is applied to the front surface of the felt, as at 4, forming a base for the 70 design coat of paint 5. This method of applying a back and a front coat without the use of sizing allows the surface to become interlocked with the fibers of the felt, and the proportions are such that the shrinkage 75 of the back and front coatings is the same as that of the felt. The design is then printed on the material by the ordinary block printing process, using a paint of such a consistency that when applied by the 80 printing blocks it will form not only the design, but also the wearing surface.

The proportions that I have used successfully for the back and front coatings of the felt are as follows:

Pigment, 1150 lb.; specially prepared linseed oil, 520 lb.; liquid drier, 100 lb.; and lead oxids 10 lb.

While I have given a certain formula, it will be understood that the formula may be 90 varied without departing from the spirit of the invention, which is to apply a surface coating to a felt body so that it will adhere to the fibers of the felt and will form a surface which will receive the paint forming the wearing surface. The proportion between the several coats and the body of the felt is such as to insure a coefficient 95 of expansion and contraction so that when the material is in the form of a rug it will 100 lie flat upon the floor and will not turn up at the edge or buckle at the center under changing conditions of the atmosphere.

I claim:

1. The process herein described of making a floor covering, said process consisting in passing a strip of felt through a semi-solid bituminous solution while the solution is hot so as to thoroughly impregnate the felt, then applying directly to one surface 110

of the felt a preparation of linseed oil, naphtha and a pigment, heating the material so as to evaporate the naphtha, cooling the same and then applying to the opposite 5 surface of the felt a similar coating and allowing it to cool, and then applying a printed design of paint to one of said surfaces.

2. The process herein described of making a floor covering, said process consisting in saturating a strip of felt forming

the base of a floor covering with a semi-solid bituminous material, applying to each face of the felt a coating of linseed oil, naphtha and a pigment, heating the material so as to evaporate the naphtha, then applying a printed design to one surface of the material, the material of each coat being such that it has the same coefficient of expansion as the base. 15

In witness whereof I affix my signature. 20  
GEORGE PRIFOLD.